

## UNITED STATES PATENT OFFICE

2,078,007

PROCESS OF MAKING ARTICLES HAVING  
THE APPEARANCE OF PEARLJacob Lurie, Springfield, Mass., assignor to The  
Fiberloid Corporation, Indian Orchard, Mass.,  
a corporation of MassachusettsNo Drawing. Application June 17, 1935,  
Serial No. 26,933

3 Claims. (Cl. 91—68)

My invention relates to the manufacture of articles having the general appearance of mother-of-pearl and similar materials whether natural or artificial, the surface of which have peculiar 5 light effects caused by the presence of minute particles either of fish scale substance or substitutes therefor, or other finely divided substances such as aluminum and bronze powders, and the so-called artificial pearl substances which reflect 10 or transmit light in different directions and in varying amounts according to their position in the material, such substances being conveniently called pearly substances. It is believed that the pearl effect from such materials is related to the 15 position of the individual particles with respect to each other, and to the surface of the sheet. In this art, this relation has been referred to as orientation. Heretofore the maximum effect has been accomplished by extruding the mixture or 20 the plastic material containing the pearly substance through a suitable orifice, then cutting the material into small pieces; laying them at random angles and compressing into a solid block which is then sheeted in the usual way.

25 I have discovered, however, that if a liquid conveniently called a carrier and containing the pearly substance is floated on the surface of a bath of another liquid, as for instance water, the particles of the pearly substance may be transferred to an article by bringing the surface of the article into contact with the surface of the carrier film as it floats on the bath, and the layer of material thus transferred to the surface of the article will have the optical effect of pearl material. The film is so flexible and plastic that it 30 conforms to the shape of the surface of the article even though it be irregular, as for example a tooth brush handle, knob or spool. The whole or only a part of the surface of the article may be 35 coated.

This process makes it possible to use a relatively small amount of the pearly substance because it is applied to the surface of the article only and is not distributed throughout the whole mass. 40 Since these pearly substances are generally expensive, this results in substantial saving. Furthermore, by choosing the color and nature of the material of which the article to be coated is made, very pleasing and unusual effects can be produced. 45 For instance, transparent plastic may be employed and this may be colored either uniformly or in varying degrees or colored, translucent, opaque or variegated materials may be employed. Likewise articles of other substances, for instance, 50 wood or metal, may be coated by my novel meth-

od. In such case, the coating may often be facilitated by the application of suitable priming coats. When desired a transparent protective coat may be applied.

5 The carrier liquid from which the film is formed is any liquid which will retain the pearly substance in suspension and will adhere to the article to be coated. In practice it is convenient to use a lacquer such as a cellulose ester or ether lacquer which may itself be transparent or may 10 be colored as required for the particular effect to be produced.

15 The pearly material in the coating may be any of a number of substances. For instance, pearl essence obtained from fish scales, certain metallic powders, such as aluminum powder, bronze powder and the like, and in fact any finely divided substance which produces the required light effect. For convenience, I employ the term pearly 20 substance to cover all such materials.

25 The bath on which the mixture of carrier liquid and pearly substance is floated is some liquid which is not a solvent for the solid constituents of the carrier liquid, although it may be miscible with one or more of the solvents used to make up the carrier liquid. For ordinary purposes water is satisfactory.

30 The article to be coated may be a sheet which is subsequently cut up or formed into the final product or it may be a completely finished article, as for instance a tooth brush handle. When a formed article is to be coated this can be done by slowly submerging the article in the bath on which the mixture is floating. When a sheet is to be 35 coated, the coating may be done by bringing the surface of the sheet progressively into contact with the mixture floating on the bath, additional coating mixture being supplied as required.

40 The nature of the ingredients of the carrier liquid affects the pattern produced; thus acetone tends to produce a more marked pearl mottle than either ethyl acetate or butyl acetate, while the addition of diluents, such as coal tar solvents, petroleum naphthas or alcohol, also changes the appearance of the mottle noticeably, and camphor 45 produces a peculiar pattern.

45 The effect of a solvent seems to vary with its rate of evaporation and the extent of its miscibility with water. This indicates that the pattern of the pearl mottle is dependent upon the interfacial forces set up between the lacquer and the water phases.

50 As an illustration of one method of practicing the process comprising my invention, the following procedure for producing sheets having a 55

pearly surface appearance may be followed. The base material, whatever that may be, is formed into a sheet or sheets of the desired size and thickness, and may even be in the form of a 5 continuous sheet or web. It may be made of transparent, translucent or opaque stock, and may be colored with varying colors as required. Very attractive effects are produced by using 10 mottled sheet stock. I then mix a transparent pyroxylin lacquer and natural pearl essence, for example in the proportion of 5 to 10 parts of essence to 100 parts of lacquer. This lacquer may be composed, for example, as follows: 1 pound of  $\frac{1}{2}$  second nitrocellulose,  $\frac{1}{3}$  pound dibutyl phthalate, and 1 gallon of solvent mixture. The solvent may be composed of the following liquids: 15 30 parts toluol, 40 parts acetone, 20 parts butyl acetate, and 10 parts ethyl acetate, all by volume. This mixture is poured slowly onto the 20 surface of a water bath. The carrier liquid, and the pearl essence which is distributed throughout 25 it, spreads out over the surface of the bath in a thin layer. The tiny particles of pearly substance in the thin coating tend to arrange themselves in patterns. After the film is formed on the bath, the surface of the sheet is brought into contact with the film thereby transferring the film with the pearly substance therein to the surface of the sheet. In practice it is desirable 30 after the coating layer has been allowed to form on the surface of the bath to allow the solvent in the coating material to evaporate somewhat thereby causing the coating to harden slightly before the article to be coated is brought in contact with it. If this is done it is also desirable to 35 soften the surface of the article to be coated by applying to it by dipping, spraying or fuming a little of a suitable solvent. This activates the surface and causes the coating to adhere more satisfactorily. In practice, I find that by this 40 procedure more satisfactory results are obtained, particularly since there is less trouble with air bubbles. This method which includes hardening a floating coating and then applying it to an article, the surface of which has preferably been 45 activated by the application of a solvent, has application to other articles than those which are to be given a pearl-like appearance and therefore is made the subject of a separate application 50 and is not claimed herein.

If an article such as a tooth brush handle, knob or spool is to be coated, the same procedure is followed except that the article, if it be of a material such as wood or metal, may be first 55 coated with a suitable primer or under coat to which the ornamental coating will adhere. The

priming or under coat may be omitted according to circumstances. After the article is prepared, the surface being activated by the application of solvent or not as required, the article is slowly submerged in the bath on which floats the ornamental coating which has preferably been allowed to harden slightly by the evaporation of solvent and preferably removed therefrom through a part of the surface of the bath which is not covered by a film. The evaporation of solvent in this case, however, should not be allowed to proceed too far. It is important that the coating be still so flexible and plastic that it conforms readily to the surface of the article and adheres strongly thereto, producing a uniform coat over the whole article. Any other convenient method of bringing the surface of the article or the portion thereof which it is desired to coat into contact with the layer of coating material floating on the surface of the bath may be employed. 20

After coating, the sheets are dried and will be found to have an excellent pearl effect with the use of a relatively small amount of pearly material. 25

The procedure employed will be substantially the same regardless of the particular pearly substance employed.

I claim:

1. The process of producing pearl effect on articles which consists in mixing the pearly substance with a suitable liquid carrier and in an amount to produce orientation, floating the mixture on a bath of liquid in a sufficiently thin film to produce orientation of the pearly substance and thereby orienting the particles of the pearly substance, and then bringing the article to be coated into contact with the mixture. 30

2. The process of making imitation pearl sheets which consists in mixing a pearly substance with a suitable carrier liquid and in an amount to produce orientation, floating the mixture on a bath of water to form a carrier film of sufficient thinness to produce orientation of the pearly substance and bringing a sheet of cellulosic material 40 into contact with the carrier film. 45

3. The process of making imitation pearl tooth brush handles which consists in mixing a pearly substance with a suitable liquid to form a carrier film and in an amount to produce orientation, floating the mixture on a bath of liquid as a sufficiently thin film to produce orientation of the pearly substance and bringing the surface of the tooth brush handle into contact with the carrier film. 50

JACOB LURIE. 55